# EUROPEAN PATENT SPECIFICATION

(11) **EP 0 624 214 B1**
(45) Date of publication and mention of the grant of the patent: **27.01.1999**
(21) Application number: 92922931.8
(22) Date of filing: 30.10.1992
(51) Int. Cl.: E01C 19/10

(54) **A METHOD OF PREPARING AN EMULSION- OR ASPHALT-CONCRETE FOR USE AS A ROAD MATERIAL**
VERFAHREN ZUM VORBEREITEN VON EINEM EMULSION- ODER ASPHALTBETON ZUR VERWENDUNG ALS STRASSENBAUMATERIAL
PROCEDE DE PREPARATION D'UN BETON EMULSIONNE OU ASPHALTIQUE UTILISE COMME MATERIAU POUR ROUTES

(30) Priority: 30.10.1991 DK 179391
(43) Date of publication of application: 17.11.1994
(73) Proprietor: Esha Holding B.V., 9744 TC Groningen (NL)
(72) Inventor: Hove, Leo, 5750 Ringe (DK)
(74) Representative: Kruk, Wiggert Johan
(86) International application number: DK9200315
(87) International publication number: WO9309295

(56) References cited:
- EP-A- 0 491 107
- WO-A-83/00700
- WO-A-87/03317
- GB-A- 334 588
- US-A- 4 978 393

## Description

The present invention relates to a method of preparing an emulsion- or asphalt-concrete for use as a road material.

It is a well known sight that asphalt concrete is laid out in a smoking hot condition, whereby it is possible to keep the mixture of stones and bitumen suitably shapable for an even laying-out and compression, just as the mixture may then have a large content of high viscid bitumen, thereby ensuring a good bonding and yet a certain, desired resiliency in the laid-out material, when its temperature decreases to ambient temperature. Only it is very energy consuming to effect the associated heating of the material.

On this background has been developed a 'cold' technique (see e.g. US-A-4 978 393), which may well have certain drawbacks or limitations, but nevertheless is considered advantageous in that the heating can be avoided. The technique is based on the use of a bitumen emulsion in admixture with a graded stone material. An aqueous bitumen emulsion has no particular bonding ability of its own, but in time a so-called 'breaking' of the emulsion occurs, whereby the emulgated bitumen fractions float together and the water is segregated, such that the bitumen may thereafter act as a binding agent that can stick to the stone surfaces and bond these together. By means of different additives it is possible to control rather accurately when this breaking should take place after the mixing operation. It is achievable, therefore, that the mixture can be prepared and transported to the laying area and be laid-out therein prior to the breaking having proceeded to the point where the material will not thereafter be suitably easily shapeable.

If the emulsion is or has not broken almost as soon as it has been laid out, one problem among others will be that in case of rain after the laying out a more or less extensive washing out of the emulsion may take place, this of course being highly unlucky or in the worst case even fatal for the work.

It is well known, therefore, that the breaking should be adjusted so as to have proceeded widely already at the time of the laying out, even though this will create the problem that it is not possible to use any particularly hard binding bitumen in the emulsion. If the breaking of an emulsion with such a hard or high viscid bitumen has proceeded widely just before the laying out, it will be impossible to effect the laying work in an easy and orderly manner under 'cold' conditions, because the material will then be so strongly bonded together that it cannot be reasonably easily shapable.

It has become a common practice that for usual applications of emulsion concrete it is only possible to use emulsions based on a relatively low viscid bitumen having a viscosity of up to some 3000 mm²/sec at 60° C. However, such materials will have a relatively poor stability, so the method is used only on roads with a low traffic load.

It could be possible to use a bitumen of a higher viscosity and even an increased amount of emulsion if care is taken that the emulsion breaks only partly during the mixing process or prior to the laying out, but also this would create serious problems. Dependent of the grain curve of the stone material it may be impossible to secure an optimal bitumen percentage, because the stone material can only 'carry' a certain amount of unbroken emulsion without surplus emulsion flowing off. Such a flow off of incompletely broken emulsion will take place during the truck transport of the material from the mixing place to the working place and thus give rise to considerable smudging problems for other road-users. Moreover, after its laying out and compaction on the road, the material will exhibit cavities holding unbroken emulsion that will cause the finished road layer, during a long period of time, to be very sensitive to rain, which causes a washing out of bitumen.

It has earlier been recognized that with a minimized, yet sufficient total amount of emulsion the problem may occur that the emulsion is predominantly 'absorbed' by the finer stone fractions, such that a required total wrapping of the coarse stones will not be achieved unless still more emulsion is added. It has been proposed to remedy this by initially supplying to the mixing stage the coarse stone fraction and the amount of emulsion necessary for a total wrapping of these stones, while the finer stone fraction is added later on, if required together with more emulsion, see e.g. US-A-923,891 and GB-A-334,588. It is possible to hereby avoid a direct waste of surplus emulsion, but there will be no resulting quality improvement of the laid out material.

It is the purpose of the invention to provide a method, by which it will be practically possible to make use of an emulsion based on a noticeably harder bitumen, i.e. a bitumen of higher viscosity, such that the laid out road layer can exhibit a considerably increased strength and yet be suitably shapeable in connection with the laying-out, without thereafter being sensible to any washing out of the bitunenous binding agent.

The invention is based on the consideration that the material as a whole will be supple and shapeable as long as the fine stone fraction has not been bonded by a high viscid bitumen, whether or not the stones in the coarse fraction have already been wrapped by a more or less broken emulsion based on a high viscid bitumen. This has lead to a further recognition of the fact that in an initial phase of the mixing process it will be possible to mix the coarse stone fraction with an emulsion based on high viscid bitumen and with an amount thereof satisfying the full wrapping need for the stones in this fraction, when this emulsion is adapted to break effectively already during the mixing process, while the finer stone fraction, also called the mortar, can be added thereafter, with further addition of emulsion, though now a different emulsion based on a low viscid bitumen, but still adapted to break no later than by the laying out of the material, that is prior to or shortly after the laying out and preferably even befor the material leaves the mixing plant.

The finally admixed emulsion will make the entire mixture supple and formable, i.e. the mixture can be laid out evenly and with ordinary equipment, although the stones of the coarse fraction have already been coated with a layer of broken, hard bonding bitumen. Because both types of emulsion are adaptable to a total or extensive breaking already before the mixture leaves the mixing plant, problems with respect to flow off during transportation to the working area will be avoided, and the laid out layer will be insensitive to rain right from the beginning.

It has been found that after the laying out a migration between the 'hard' bitumen on the coarse stones and the 'soft' bitumen in the finer stone fraction will take place rather soon, such that the result will be a total bonding obtained quicker and with a more high viscid and therewith better binding bitumen than so far known or achievable.

Thus, also in the process of the invention there is made use of the respective coarse and fine stone fractions, but now with addition of the crucial circumstance that the two fractions are treated with respective, very different emulsions.

The principle of the invention may be advantageously used also for the production of an asphalt material in which the binding agent is bitumen in non-emulgated condition. Here the coarse stone fraction is heated to such a high temperature, by which the stones can be totally coated by the initially added high viscid bitumen, which, itself; is heated to assume a viscosity suitably low for this purpose. Thereafter the fine fraction is added to the mixer, in either cold or warm condition all according to the applied low viscid bitumen, which is also added; this bitumen should have a temperature high enough to condition such a low viscosity that the bitumen can effectively coat the stone particles of the fine fraction. This temperature should be somewhat lower than the temperature of the coarse fraction, such that the coating of the coarse stones by the high viscid bitumen will be stabilized.

Generally, with the considered method it is possible to work with a very high viscid bitumen for the initial mixing with the coarse stone fraction, just when care is taken that the fine fraction is not added until an extensive coating of the coarse stones has been obtained. As far as the emulsion concrete is concerned it is important that the relevant 'hard' emulsion is widely broken before the fine fraction and the associated 'soft' emulsion is added, but it is a lucky coincidence that the very addition of the fine stone fraction, with its very large surface area, strongly promotes the breaking of the hard emulsion, such that the latter will break finally almost automatically at an ideal moment of the process. With the hot method it is sufficient to use a moderate heating, as the high viscid bitumen shall not be conditioned to be mixed with the fine stone fraction. All according to the application purpose this bitumen has a viscosity in the range of 5000 - 75000 mm²/sec at 60° C.

With the use of the 'soft' emulsion or the low viscid bitumen, respectively, in connection with the fine stone fraction it is possible to achieve a homogenous admixture into the fine fraction, also here without any extensive heating as far as the hot method is concerned. The viscosity of the relevant bitumen should normally be somewhat lower that 3000 mm²/sec, but under special circumstances this figure may be higher, up to 4-5000, though still noticeably smaller than the viscosity figure of the applied high viscid bitumen.

The weight ratio between the two kinds of bitumen may vary all according to the dispensary of the material mixture, but a typical ratio can be 60%PC% high viscid and 40%PC% low viscid bitumen. Already some 24 hours after the laying out of the material an equalization of the viscosities will have taken place, and on this background it is perfectly possible, if desired, to obtain resulting viscosity figures of MB 10-30.000, this being unheard in connection with conventional emulsion concrete and very expensively achievable in other conventional asphalt preparation.

The applied mixing plant can be a simple batch mixer or a continuous throughflow mixer, but it would be possible to use separate mixers for the mixing of the respective binding agents into the respective stone fractions and a separate mixer for the bringing together of the thus pretreated fractions.

When preparing the emulsion concrete it will be advantageous to control the breaking of the 'hard' emulsion such that it will break as soon as a practically total wrapping of the coarse stones has taken place, e.g. after a mixing time of 10-12 seconds, such that this emulsion will not get time to be 'diluted' with the subsequently added 'softer' emulsion as added in connection with the addition of the fine stone fraction. Thereby the hard emulsion can be dosed in accordance with the desired maximum carrying capacity of the stones of the coarse fraction, while a dilution of the emulsion would cause a weakening of this carrying capacity and thereby of the possibility of an efficient exploitation of the high viscid bitumen.

Another important effect of the rapid addition of the fine stone fraction as soon as the hard emulsion has been distributed and broken is that by this addition an advanced adhesion between the stones of the coarse fraction will be prevented, which could otherwise give rise to undesired lump formations. In practice it is correspondingly important that the breaking of the added 'soft' emulsion takes place no later than by the finishing and delivering of the material mixture from the mixing plant, in order to thereby counteracing later problems with respect to washing out of the emulsion after the laying out of the material or already during the transportation thereof to the working place. It is less important whether the soft emulsion is added briefly before, concurrently with, or briefly after the addition of the fine stone fraction.

It is essential to notice that the very controlling of the breaking time of the applied emulsions belongs to already well established art, such that this will not have to be further elucidated in the present connection.

In connection with the invention it will be possible to pretreat the coarse stone fraction with the emulsion containing the high viscid bitumen, while by the addition of the fine stone fraction there is not used any emulsion, but a bitumenous binding agent having a quite low viscosity, e.g MB 1500-2000 at 60° C. This additive may be administered in cold condition, and it will render the material well shapeable. In so far as the migration with the high viscid bitumen will take place soon after the laying out, a desirable result will be achievable also in this manner, even when the resulting bitumen percentage of the material may be still higher by the use of the 'soft' emulsion for the fine stone fraction.

Hereafter a few examples of dispensaries according to the invention should be given:

### Example 1:

Stone material: 60 weight percent of 4-16 mm coarse fraction,
40%PC% weight percent of 0-4 mm fine fraction.
Binding agent emulsion: Type 1: BE65R/20.000
Type 2: BE65M/3.000.

In these denominations, "BE" stands for "bitumen emulsion", "65" for the admixtury percentage of the bitumen, "R" for a rapidly breaking emulsion, "M" for a medium breaking emulsion, and the figure indications 20.000 and 3.000 for the viscosity of the respective bitumens, measured by mm²/sec. at 60° C.

By experiments it is established that the breaking time for the emulsion type 1 on the coarse fraction type of atones is a certain amount of seconds, e.g. 12-14 seconds. The coarse fraction is introduced currently and without heating into a flow-through mixer, at the entrance end of which the emulsion of the said type 1 is added by a flow corresponding to a weight amount of 7-8 %PC% of the stone weight. In the mixer the aqueous solution of the emulsion will be distributed evenly around the atones in few seconds. At a following place of the mixer, corresponding to a material transportation time of 14-16 seconds, a flow of the fine stone fraction and emulsion type 2 at a weight ratio of some 100:8 is added. The total product is conveyed further in the mixer for intensive mixing through additional 20-30 seconds, corresponding approximately to the breaking time of the emulsion type 2, whereafter the mixture is let out in a flow to a carrier truck. The truck takes the collected material portion to a delivery apparatus at the working site, where the laying out is effected not later than 4-5 hours after the preparation of the material mixture. In the laid out emulsion concrete there will be a residual bitumen percentage of approximately 5.

### Example 2:

Stone material: 60 weight percent of 5-18 mm coarse fraction
40 weight percent of 0-5 mm fine fraction.
Binding agent: Type 1: B 180
Type 2: MB 3.000

In these denominations "B" stands for a pure or non-emulgated bitumen, while the figure 180 refers to a penetration of 180 at 25° C, corresponding to a viscosity of some 60.000 mm²/sec at 60° C. MB 3.000 denotes the non-emulgated bitumen having a viscosity of 3.000 mm²/sec at 60° C.

1800 kg stones of the coarse fraction heated to some 130° C is filled into a charge mixer, and after start of the mixer 90 kg binding agent type 1, heated to some 130° C is added. 8-12 seconds thereafter 1200 kg of the fine fraction is added, this fraction not having to be heated, and also 60 kg binding agent type 2, heated to roughly 90° C. When the mixture portion of about 3 tons has been homogeneously mixed, e.g. after 25 seconds, the charge is let out to a carrier truck, and care is taken that the mixture is laid out not more than 5-6 hours after its preparation. The delivery temperature in the mixer can be some 60° C.

## Claims

1. A method of preparing an emulsion concrete or asphalt concrete to be laid out as a road material, comprising the following steps:
- selecting a coarse stone fraction and a fine stone fraction,
- coating the coarse stone fraction with a first bitumen of a relatively high viscosity in the range of 5000-75.000 mm²/sec at 60°C, by one of the steps a) or b) :
a) mixing the coarse stone fraction with a first bitumen emulsion based on said high viscid first bitumen and prepared for breaking not later than by a following addition of the fine stone fraction,
b) mixing the coarse stone fraction in heated condition with said high viscid first bitumen also in a heated condition,
- adding to that mixture said fine stone fraction and a second bitumen of a relatively low viscosity being lower than 5000 mm²/sec at 60°C, and substantially lower than the viscosity of said first bitumen, by one of the steps c) or d) :
c) mixing the fine stone fraction, integrated in the mixing with the coarse stone fraction, with a second bitumen emulsion based on said low viscid second bitumen and prepared for breaking before a following laying out of the concrete material,
d) mixing the fine stone fraction, integrated in the mixing with the coarse stone fraction, with said low viscid second bitumen in a cold or heated condition, yet when used in combination with the above step b) being heated to a temperature below the temperature used in that step b),
- mixing all said ingredients for effectively preventing short term clogging of the coarse stone fraction, and
- bringing out the mixed material prior to the same setting by migration of the first and second bitumen.

2. A method according to claim 1, in which the first bitumen for the coarse stone fraction is of a viscosity of at least 20.000 mm²/sec at 60°C.

3. A method according to claim 1, in which the second bitumen for use in said step d) is a bitumen of a viscosity in the range of 1500-2000 mm²/sec at 60°C.

4. A method according to claim 1, in which said step a) is effected such that the breaking of the first bitumen emulsion takes place as soon as the coarse stones are fully coated with the emulsion.

5. A method according to claim 1, whereby the second bitumen emulsion is prepared so as to break shortly after or even prior to the mixed material leaving the mixing station, for urgent use of the mixture.

6. An emulsion concrete or asphalt concrete prepared in accordance with the method of claim 1, exhibiting a resulting bitumen viscosity in the range of 10000-30000 mm²/sec. at 60°C.

## Patentansprüche

1. Verfahren zur Herstellung eines als Straßenbaumaterial verlegbaren Emulsionsbetons oder Asphaltbetons, umfassend die folgenden Schritte:
- Auswählen einer groben Steinfraktion und einer feinen Steinfraktion,
- Beschichten der groben Steinfraktion mit einem ersten Bitumen einer relativ hohen Viskosität im Bereich von 5000 - 75 000 mm²/s bei 60 °C durch einen der Schritte a) oder b) :
a) Vermischen der groben Steinfraktion mit einer ersten Bitumenemulsion auf der Grundlage des hochviskosen ersten Bitumens, die so hergestellt wird, daß sie nicht später als nach einer nachfolgenden Zugabe der feinen Steinfraktion bricht,
b) Vermischen der groben, in einem erwärmten Zustand befindlichen Steinfraktion mit dem ersten hochviskosen, ebenfalls in einem erwärmten Zustand befindlichen Bitumen,
- Zugeben der feinen Steinfraktion und eines zweiten Bitumens mit einer relativ niedrigen Viskosität, die niedriger als 5000 m²/s bei 60 °C und wesentlich niedriger als die Viskosität des ersten Bitumens ist, zu dieser Mischung durch einen der Schritte c) oder d):
c) Vermischen der in die Mischung mit der groben Steinfraktion einzuarbeitenden feinen Steinfraktion mit einer zweiten Bitumenemulsion auf der Grundlage des zweiten, niedrigviskosen Bitumens, die so hergestellt wird, daß sie bricht, bevor das Betonmaterial anschließend verlegt wird,
d) Vermischen der in die Mischung mit der groben Steinfraktion einzuarbeitenden feinen Steinfraktion mit dem zweiten, in einem kalten oder erwärmten Zustand befindlichen, niedrigviskosen Bitumen, der jedoch, wenn er in Kombination mit dem obigen Schritt b) verwendet wird, auf eine Temperatur erwärmt wird, die niedriger als die in Schritt b) angewandte Temperatur ist,
- Vermischen aller Bestandteile, damit eine kurzfristige Klumpenbildung der groben Steinfraktion verhindert wird, und das
- Ausbringen des gemischten Materials, bevor dieses durch die Migration des ersten und zweiten Bitumens erhärtet.

2. Verfahren nach Anspruch 1, wobei der erste Bitumen für die grobe Steinfraktion eine Viskosität von wenigstens 20 000 mm²/s bei 60 °C aufweist.

3. Verfahren nach Anspruch 1, wobei der zweite Bitumen zur Verwendung in Schritt b) ein Bitumen mit einer Viskosität im Bereich von 1500 - 2000 mm²/s bei 60 °C ist.

4. Verfahren nach Anspruch 1, wobei Schritt a) so bewerkstelligt wird, daß das Brechen der ersten Bitumenemulsion erfolgt, sobald die groben Steine vollständig mit der Emulsion beschichtet sind.

5. Verfahren nach Anspruch 1, wobei die zweite Bitumenemulsion so hergestellt wird, daß sie kurze Zeit, nachdem das gemischte Material die Mischanlage verläßt, oder sogar davor bricht, damit die Mischung kurzfristig eingesetzt werden kann.

6. Emulsionsbeton oder Asphaltbeton, hergestellt gemäß dem Verfahren von Anspruch 1, der eine resultierende Bitumenviskosität im Bereich von 10 000 - 30 000 mm²/s bei 60 °C aufweist.

## Revendications

1. Procédé pour préparer un béton en émulsion ou un béton asphaltique à étaler en tant que matériau routier, comprenant les étapes suivantes:
- sélection d'une fraction de gravillons grossiers et d'une fraction de gravillons fins,
- revêtement de la fraction de gravillons grossiers avec un premier bitume d'une viscosité relativement élevée dans la gamme comprise entre 5000 et 75000 mm²/sec à 60°C, selon l'une des étapes a) ou b) :
a) mélange de la fraction de gravillons grossiers avec une première émulsion de bitume, à base dudit premier bitume de viscosité élevée, et préparée pour obtenir la rupture de l'émulsion au plus tard lors de l'addition ultérieure de la fraction de gravillons fins,
b) mélange de la fraction de gravillons grossiers à l'état chaud avec ledit premier bitume de viscosité élevée également à l'état chaud,
- addition à ce mélange de ladite fraction de gravillons fins et d'un second bitume d'une viscosité relativement faible, inférieure à 5000 mm²/sec à 60°C et substantiellement inférieure à la viscosité dudit premier bitume, selon l'une des étapes c) ou d):
c) mélange de la fraction de gravillons fins, intégrée dans le mélange avec la fraction de gravillons grossiers, avec une seconde émulsion de bitume, à base dudit second bitume de faible viscosité, et préparée pour obtenir la rupture de l'émulsion avant la pose ultérieure du matériau de béton,
d) mélange de la fraction de gravillons fins, intégrée dans le mélange avec la fraction de gravillons grossiers, ledit second bitume de faible viscosité étant à l'état froid ou chaud, mais, lorsqu'on l'utilise en combinaison avec l'étape b) ci-dessus celui-ci est chauffé à une température inférieure à la température utilisée dans l'étape b),
- mélange de tous lesdits ingrédients afin d'éviter d'une manière efficace le colmatage à court terme de la fraction de gravillons fins et,
- le déchargement du matériau mélangé avant la prise par migration du premier et du second bitume.

2. Procédé selon la revendication 1, dans lequel le premier bitume pour la fraction de gravillons grossiers présente une viscosité d'au moins 20 000 mm²/sec à 60°C.

3. Procédé selon la revendication 1, dans lequel le second bitume que l'on utilise dans ladite étape d) est un bitume d'une viscosité comprise dans la gamme entre 1500 et 2000 mm²/sec à 60°C.

4. Procédé selon la revendication 1, dans lequel ladite étape a) est effectuée de telle sorte que la rupture de la première émulsion de bitume ait lieu dès que les gravillons grossiers sont totalement enrobés par l'émulsion.

5. Procédé selon la revendication 1, dans lequel la second émulsion de bitume est préparée de manière à se rompre peu après ou même avant que le matériau mélangé ne quitte la station de mélange, pour une utilisation urgente du mélange.

6. Béton en émulsion ou béton asphaltique préparé selon le procédé de la revendication 1, présentant une viscosité de bitume résultante dans la gamme comprise entre 10000 et 30000 mm²/sec à 60°C.
